

1

3,293,062

CHEMICAL WATERMARK APPLIED ON  
FINISHED PAPER

Bruce D. Skofronick and Frans V. E. Vaurio, Appleton, Wis., assignors, by mesne assignments, to Customark Corporation, Appleton, Wis., a corporation of Wisconsin

No Drawing. Filed Apr. 5, 1963, Ser. No. 270,826  
10 Claims. (Cl. 117—38)

This invention relates to a method of placing a chemical watermark in finished blank paper.

It is an expensive procedure to place watermarks in paper when done while a paper web is being formed. Obviously, a small order for watermarked paper is prohibitively expensive.

This disadvantage has been overcome by providing chemical watermarks which are applied to the finished blank papers. Such a process has been set out in copending application, Serial No. 78,228, filed December 27, 1960, now U.S. 3,140,959.

An object of this invention is a method for making chemical watermarks which are substantially insoluble and colorless.

Another object is a method for making chemical watermarks by applying a liquid chemical composition to the surface of finished paper and then curing the composition in the paper.

Another object is a method which makes watermarked paper economically and easily available.

Another object is a method which provides great versatility in the available watermark designs which can be placed in finished paper.

Another object is a method for simply and efficiently making chemical watermarks substantially at room temperature to thereby eliminate any necessity of involved procedure steps or high temperature cures.

Another object is a method for making a watermark in finished paper with a composition containing a chemical which cures into a colorless, substantially insoluble watermark design.

Another object is a method for making watermarks with a composition having resins combined with a chemical compound which together cure to a substantially insoluble, colorless and transparent watermark design.

Another object is a finished blank paper having a watermark applied by the foregoing methods.

A chemical watermark is successful if it is substantially insoluble, it doesn't have a gloss, it is colorless, it can survive under aging, it has good ink receptivity and the like, and it does not damage the finished paper. Such a successful watermark is made by applying a generally liquid composition in the configuration of a selected design to the surface of finished paper. It has been found that hexamethoxymethylmelamine, which is supplied under the trademark Cymel 300 by the American Cyanamid Company, can be combined with other ingredients to make a composition having the foregoing desirable features. Hexamethoxymethylmelamine has the following chemical structure:



It is surprising that hexamethoxymethylmelamine makes a successful watermark since this material is not generally considered to be a resin in the sense that cross-linking can occur. Whatever the mechanism which occurs

2

may be, it has been found that hexamethoxymethylmelamine in combination with acid curing agents, such as alkyl and aryl sulfonic acid derivatives, does harden into a colorless, substantially insoluble watermark in finished paper.

5 Alkyl substituted aryl sulfonic acids may be ortho, meta and paratoluene sulfonic acid; alkyl sulfonic acids such as methane sulfonic acids and ethane sulfonic acids are also useful as well as the di- and tri-alkyl substituted phenyl sulfonic acids. The o- and p-toluene sulfonic acids are excellent curing agents. Where the curing agent is identified merely as "toluene sulfonic acid" in the following examples, it is intended to represent a mixture of about 80 percent p-toluene sulfonic acid and about 20 percent o-toluene sulfonic acid.

10 The combination of hexamethoxymethylmelamine with such curing agent may alone form a useful composition, but it is preferred to add a colorless, organic solvent to the composition. The preferred solvents are polar solvents such as glycol ethers, ketones, and like polar solvents. A widely adaptable solvent is diethyleneglycol monomethyl ether which will conveniently be referred to as methyl "Carbitol."

15 The concentrations of the ingredients in the compositions can be varied within liberal ranges to obtain good quality chemical watermarks. It has been found that compositions containing from about 3-15 percent by weight of curing agent and from about 40-60 percent by weight of solvent provide workable compositions leading to good quality chemical watermarks. It has been further found that if the amount of curing agent is increased to about 20 percent by weight a good quality chemical watermark is provided after a short period of aging, say about 5-15 days.

20 30 35 40 Other ingredients and resins may be added to the compositions shown here to obtain chemical watermarks having modified physical and chemical characteristics. It has, for example, been found that epoxy resins may be added to a composition of hexamethoxymethylmelamine, curing agent and solvent to obtain excellent chemical watermarks.

45 The following examples are set forth to illustrate various embodiments of the invention, but such examples should not be considered as an exclusive representative and teaching of the practice of the invention.

*Example I*

Four different compositions containing different amounts of the ingredients, by weight, were prepared as follows:

| Composition | Hexamethoxy-methylmelamine, Percent | Toluene sulfonic acid, Percent | Methyl "Carbitol," Percent |
|-------------|-------------------------------------|--------------------------------|----------------------------|
| 1-----      | 50                                  | 20                             | 30                         |
| 2-----      | 52                                  | 28                             | 20                         |
| 3-----      | 70                                  | 20                             | 10                         |
| 4-----      | 80                                  | 20                             | 0                          |

55 60 65 70 75 The ingredients were combined substantially at room temperature in each of the separate compositions. A small amount of each composition was spread uniformly over a glass surface with a conventional hand roller. A hand stamp, having a design of selected configuration made from rubber-like material, was pressed against the wet film and then stamped on the surface of a finished sheet of paper. Several separately stamped sheets were prepared for each of the compositions. Watermarks less than 5 days old were soluble in water, ethyl alcohol, carbon tetrachloride and acetone. Watermarks aged longer than 5 days were insoluble in all of the foregoing solvents.

Side-by-side compositions identified as A and B were prepared by varying concentrations of ingredients. The only difference was that Composition A contained hexamethoxymethylmelamine whereas Composition B contained melamine formaldehyde, a well-known curable

COH, C=O, CCl<sub>4</sub>, and H<sub>2</sub>O. The solvent resistance of the marks was graded as either good (G) or not good (NG). Un-aged sheets containing marks were held at room temperature for a minimum period of 24 hours and un-aged sheets containing marks were held in an oven at 105 degrees C. for 15 minutes. Table 1 sets forth the results.

TABLE 1

| Comparison           | 1                 |                   |                   |                   | 2                 |                   |                   |                   | 3                 |                   |                   |                   |        |
|----------------------|-------------------|-------------------|-------------------|-------------------|-------------------|-------------------|-------------------|-------------------|-------------------|-------------------|-------------------|-------------------|--------|
|                      | A                 |                   | B                 |                   | A                 |                   | B                 |                   | A                 |                   | B                 |                   |        |
| Composition          | Percent by weight | Percent by weight | Percent by weight | Percent by weight | Percent by weight | Percent by weight | Percent by weight | Percent by weight | Percent by weight | Percent by weight | Percent by weight | Percent by weight |        |
| Compound             | 54.4              | 54.4              | 36.5              | 36.5              | 46.3              | 46.3              | 36.5              | 36.5              | 46.3              | 46.3              | 13.9              | 13.9              |        |
| Curing Agent         | 5.4               | 5.4               | 3.6               | 3.6               | 9.2               | 9.2               | 3.6               | 3.6               | 9.2               | 9.2               | 39.8              | 39.8              |        |
| Solvent              | 40.2              | 40.2              | 59.9              | 59.9              | 60.1              | 60.1              | 59.9              | 59.9              | 60.1              | 60.1              | None              | None              |        |
| Gloss                | None              | None              | None              | None              | None              | None              | Good              | Poor              | Good              | Good              | None              | None              |        |
| Distinction          | Good              | Fair              | Good              | Poor              | Poor              | Poor              | 5                 | 30                | 30                | 30                | Fair              | Fair              |        |
| Penetration, Seconds | 10                | 25                | 10                | 5                 | 30                | 30                | 30                | 30                | 30                | 30                | 30                | 30                |        |
| Solvent Resistance:  |                   | Aged              | Unaged            | Aged              | Unaged            | Aged              | Unaged            | Aged              | Unaged            | Aged              | Unaged            | Aged              | Unaged |
| COH                  | G                 | G                 | G                 | NG                | G                 | G                 | G                 | G                 | NG                | G                 | NG                | G                 | NG     |
| C=O                  | G                 | G                 | G                 | NG                | G                 | G                 | G                 | G                 | NG                | G                 | NG                | G                 | NG     |
| CCl <sub>4</sub>     | G                 | G                 | G                 | NG                | G                 | G                 | G                 | G                 | NG                | G                 | NG                | G                 | NG     |
| H <sub>2</sub> O     | G                 | G                 | G                 | NG                | G                 | G                 | G                 | G                 | NG                | G                 | NG                | G                 | NG     |

resin. The compositions contained the following ingredients:

| A                                                                          | B                                                                      |
|----------------------------------------------------------------------------|------------------------------------------------------------------------|
| Hexamethoxymethylmelamine.<br>Toluene sulfonic acid.<br>Methyl "Carbitol." | Melamine formaldehyde.<br>Toluene sulfonic acid.<br>Methyl "Carbitol." |

In the table, the percent figures are listed to correspond with the foregoing order of ingredients. The ingredients are identified in the table simply as compound, curing agent and solvent.

The marks were evaluated for gloss in terms of "none" or "present."

Penetration was evaluated in number of seconds required for a mark to lose its surface gloss.

It is seen from the foregoing table that the compositions containing hexamethoxymethylmelamine possess the desirable features of a chemical watermark whereas the compositions containing melamine formaldehyde do not.

Table 2 sets forth data from similar compositions which differ only in that the curing agent is paratoluene sulfonic acid rather than toluene sulfonic acid mixture. The A and B compositions are identified as follows:

| A                                                                               | B                                                                           |
|---------------------------------------------------------------------------------|-----------------------------------------------------------------------------|
| Hexamethoxymethylmelamine.<br>Para-toluene sulfonic acid.<br>Methyl "Carbitol." | Melamine formaldehyde.<br>Para-toluene sulfonic acid.<br>Methyl "Carbitol." |

In the table, the percent figures are listed to correspond with the foregoing order of ingredients.

| Comparison           | 1                 |                   |                   |                   | 2                 |                   |                   |                   | 3                 |                   |                   |                   |        |
|----------------------|-------------------|-------------------|-------------------|-------------------|-------------------|-------------------|-------------------|-------------------|-------------------|-------------------|-------------------|-------------------|--------|
|                      | A                 |                   | B                 |                   | A                 |                   | B                 |                   | A                 |                   | B                 |                   |        |
| Composition          | Percent by weight | Percent by weight | Percent by weight | Percent by weight | Percent by weight | Percent by weight | Percent by weight | Percent by weight | Percent by weight | Percent by weight | Percent by weight | Percent by weight |        |
| Compound             | 54.4              | 54.4              | 33.3              | 33.3              | 30.7              | 30.7              | 33.3              | 33.3              | 30.7              | 30.7              | 9.2               | 9.2               |        |
| Curing Agent         | 5.4               | 5.4               | 6.7               | 6.7               | 60.1              | 60.1              | 60.0              | 60.0              | 60.1              | 60.1              | 60.1              | 60.1              |        |
| Solvent              | 40.2              | 40.2              | 60.0              | 60.0              | None              | None              | None              | None              | None              | None              | Good              | Good              |        |
| Gloss                | None              | None              | Good              | Good              | Poor              | Poor              | Poor              | Poor              | None              | None              | Poor              | Poor              |        |
| Distinction          | Good              | Fair              | 7                 | 7                 | 10                | 10                | 20                | 20                | 10                | 10                | 10                | 10                |        |
| Penetration, Seconds | 15                | 30                | 7                 | 7                 | 30                | 30                | 30                | 30                | 30                | 30                | 30                | 30                |        |
| Solvent Resistance:  |                   | Aged              | Unaged            | Aged              | Unaged            | Aged              | Unaged            | Aged              | Unaged            | Aged              | Unaged            | Aged              | Unaged |
| COH                  | G                 | G                 | G                 | NG                | G                 | G                 | NG                | NG                | G                 | G                 | NG                | G                 | NG     |
| C=O                  | G                 | G                 | G                 | NG                | G                 | G                 | NG                | NG                | G                 | G                 | NG                | G                 | NG     |
| CCl <sub>4</sub>     | G                 | G                 | G                 | NG                | G                 | G                 | NG                | NG                | G                 | G                 | NG                | G                 | NG     |
| H <sub>2</sub> O     | G                 | G                 | G                 | NG                | G                 | G                 | NG                | NG                | G                 | G                 | NG                | G                 | NG     |

The distinction of the mark was rated as good, fair, or poor. The distinction evaluation particularly relates to the clarity of the mark.

The solvent resistance of the mark was rated against four solvents, namely, alcohol, acetone, carbon tetrachloride, and water, which were respectively identified as

Example III

Side-by-side compositions identified as A and B were prepared with varying concentrations of the ingredients. The only difference is that A contains hexamethoxymethylmelamine whereas B contains melamine formaldehyde, a well-known curable resin. An epoxy resin, Dow DER-

supplied by Dow Chemical Company, was added to each composition. The compositions contained the following ingredients:

| A                                                                                      | B                                                                                  |
|----------------------------------------------------------------------------------------|------------------------------------------------------------------------------------|
| Hexamethoxymethylmelamine.<br>Dow DER.<br>Toluene sulfonic acid.<br>Methyl "Carbitol." | Melamine formaldehyde.<br>Dow DER.<br>Toluene sulfonic acid.<br>Methyl "Carbitol." |

The chemical watermarks were evaluated and graded as in Table 2. Table 3 sets forth the results.

McGraw-Hill, New York; and various U.S. patents, among which may be mentioned Patent Nos. 2,712,535; 2,864,775; and 2,964,694.

The compositions containing the epoxy resins are successfully used when there is present about 12-3 percent, by weight, of curing agent, and 60-10 percent of solvent. A variety of organic solvents may be used since it is only required that the chemical ingredients be soluble in the solvent, colorless and non-corrosive to the finished paper. The solvent also has a vapor pressure at room temperature sufficiently high to quickly evaporate so the ingredients in the composition do not unduly migrate and there-

TABLE 3

| Comparison           | 1                 |                   |                   |                   | 2                 |                   |                   |                   | 3                 |                   |                   |                   |
|----------------------|-------------------|-------------------|-------------------|-------------------|-------------------|-------------------|-------------------|-------------------|-------------------|-------------------|-------------------|-------------------|
|                      | A                 |                   | B                 |                   | A                 |                   | B                 |                   | A                 |                   | B                 |                   |
| Composition          | Percent by weight | Percent by weight | Percent by weight | Percent by weight | Percent by weight | Percent by weight | Percent by weight | Percent by weight | Percent by weight | Percent by weight | Percent by weight | Percent by weight |
| Compound             | 52.6              | 52.6              | 36.3              | 36.3              | 60.5              | 60.5              | 69.5              | 69.5              |                   |                   |                   |                   |
| Resin                | 31.6              | 31.6              | 26.7              | 26.7              | 13.8              | 13.8              | 13.8              | 13.8              |                   |                   |                   |                   |
| Solvent              | 10.5              | 10.5              | 40.0              | 40.0              | 9.7               | 9.7               | 9.7               | 9.7               |                   |                   |                   |                   |
| Curing agent         | 5.3               | 5.3               | 3.7               | 3.7               | 7.0               | 7.0               | 7.0               | 7.0               |                   |                   |                   |                   |
| Gloss                | None              | Not compatible    | None              | None              | None              | None              | Not compatible    | Not compatible    |                   |                   |                   |                   |
| Distinction          | Good              | Not compatible    | Good              | Good              | Good              | Good              | Not compatible    | Not compatible    |                   |                   |                   |                   |
| Penetration, Seconds | 300               | Not compatible    | 30                | 15                | 300               | 300               | Not compatible    | Not compatible    |                   |                   |                   |                   |
|                      | Aged              | Unaged            | Aged              | Unaged            | Aged              | Unaged            | Aged              | Unaged            | Aged              | Unaged            | Aged              | Unaged            |
| Solvent Resistance:  |                   |                   |                   |                   |                   |                   |                   |                   |                   |                   |                   |                   |
| CO <sub>2</sub>      | G                 | NG                | Not compatible    |                   | G                 | NG                | G                 | NG                | G                 | NG                | G                 | NG                |
| C=O                  | G                 | NG                |                   |                   | G                 | NG                | G                 | NG                | G                 | NG                | G                 | NG                |
| CCl <sub>4</sub>     | G                 | NG                |                   |                   | G                 | NG                | G                 | NG                | G                 | NG                | G                 | NG                |
| H <sub>2</sub> O     | G                 | G                 |                   |                   | G                 | NG                | G                 | NG                | G                 | NG                | G                 | NG                |
| Comparison           | 4                 |                   |                   |                   | 5                 |                   |                   |                   | 6                 |                   |                   |                   |
| Composition          | A                 |                   | B                 |                   | A                 |                   | B                 |                   | A                 |                   | B                 |                   |
|                      | Percent by weight | Percent by weight | Percent by weight | Percent by weight | Percent by weight | Percent by weight | Percent by weight | Percent by weight | Percent by weight | Percent by weight | Percent by weight | Percent by weight |
| Compound             | 46.2              | 46.2              | 31.6              | 31.6              | 26.1              | 26.1              | 26.1              | 26.1              |                   |                   |                   |                   |
| Resin                | 9.2               | 9.2               | 19.0              | 19.0              | 26.1              | 26.1              | 26.1              | 26.1              |                   |                   |                   |                   |
| Solvent              | 40.0              | 40.0              | 39.9              | 39.9              | 40.0              | 40.0              | 40.0              | 40.0              |                   |                   |                   |                   |
| Curing agent         | 4.6               | 4.6               | 9.5               | 9.5               | 7.8               | 7.8               | 7.8               | 7.8               |                   |                   |                   |                   |
| Gloss                | None              | None              | None              | None              | None              | None              | None              | None              |                   |                   |                   |                   |
| Distinction          | Good              | Fair              | Fair              | Fair              | Good              | Good              | Good              | Good              |                   |                   |                   |                   |
| Penetration, Seconds | 25                | 10                | 30                | 13                | 60                | 60                | 60                | 60                |                   |                   |                   |                   |
|                      | Aged              | Unaged            | Aged              | Unaged            | Aged              | Unaged            | Aged              | Unaged            | Aged              | Unaged            | Aged              | Unaged            |
| Solvent Resistance:  |                   |                   |                   |                   |                   |                   |                   |                   |                   |                   |                   |                   |
| CO <sub>2</sub>      | G                 | G                 | G                 | NG                | G                 | G                 | G                 | NG                | G                 | NG                | G                 | NG                |
| C=O                  | G                 | G                 | G                 | NG                | G                 | G                 | G                 | NG                | G                 | NG                | G                 | NG                |
| CCl <sub>4</sub>     | G                 | G                 | G                 | G                 | G                 | G                 | G                 | NG                | G                 | NG                | G                 | NG                |
| H <sub>2</sub> O     | G                 | G                 | G                 | G                 | G                 | G                 | G                 | NG                | G                 | NG                | G                 | NG                |
| Comparison           | 7                 |                   |                   |                   | 8                 |                   |                   |                   | 9                 |                   |                   |                   |
| Composition          | A                 |                   | B                 |                   | A                 |                   | B                 |                   | A                 |                   | B                 |                   |
|                      | Percent by weight | Percent by weight | Percent by weight | Percent by weight | Percent by weight | Percent by weight | Percent by weight | Percent by weight | Percent by weight | Percent by weight | Percent by weight | Percent by weight |
| Compound             | 40.0              | 40.0              | 19.0              | 19.0              | 23.6              | 23.6              | 23.6              | 23.6              |                   |                   |                   |                   |
| Resin                | 8.0               | 8.0               | 31.6              | 31.6              | 14.2              | 14.2              | 14.2              | 14.2              |                   |                   |                   |                   |
| Solvent              | 40.0              | 40.0              | 39.9              | 39.9              | 59.8              | 59.8              | 59.8              | 59.8              |                   |                   |                   |                   |
| Curing agent         | 12.0              | 12.0              | 9.5               | 9.5               | 3.4               | 3.4               | 3.4               | 3.4               |                   |                   |                   |                   |
| Gloss                | None              | None              | None              | None              | None              | None              | None              | None              |                   |                   |                   |                   |
| Distinction          | Good              | Fair              | Fair              | Fair              | Fair              | Fair              | Fair              | Fair              |                   |                   |                   |                   |
| Penetration, Seconds | 30                | 15                | 25                | 8                 | 20                | 20                | 20                | 20                |                   |                   |                   |                   |
|                      | Aged              | Unaged            | Aged              | Unaged            | Aged              | Unaged            | Aged              | Unaged            | Aged              | Unaged            | Aged              | Unaged            |
| Solvent Resistance:  |                   |                   |                   |                   |                   |                   |                   |                   |                   |                   |                   |                   |
| CO <sub>2</sub>      | G                 | G                 | G                 | NG                | G                 | NG                | G                 | NG                | G                 | NG                | G                 | NG                |
| C=O                  | G                 | G                 | G                 | NG                | G                 | NG                | G                 | NG                | G                 | NG                | G                 | NG                |
| CCl <sub>4</sub>     | G                 | G                 | G                 | G                 | G                 | G                 | G                 | NG                | G                 | NG                | G                 | NG                |
| H <sub>2</sub> O     | G                 | G                 | G                 | NG                | G                 | NG                | G                 | NG                | G                 | NG                | G                 | NG                |

The epoxy resins used in the previous example may be any of the reaction products of bisphenol A and epichlorohydrin. Such resins are well known and are described in the text *Epoxy Resins* by Lee and Neville (1957), 75

by alter the design of selected configuration. The vapor pressure should, however, be low enough to allow the ingredients in the composition to penetrate into the paper. Among useful solvents are ketones, such as methyliso-

butylketone, cyclohexane; esters, such as ethyl lactate, dibutyl phthalate, and N-butyl acetate; glycol ethers, such as ethyleneglycol monomethyl ether, etheneglycol dimethyl ether, diethyleneglycol monomethyl ether; and other solvents, such as dimethyl formamide, dimethylsulfoxide, and triacetin.

We claim:

1. A method for making a colorless, substantially insoluble watermark in finished paper which includes the steps of applying to the surface of finished paper a composition having curable hexamethoxymethylmelamine and a curing agent therefor which is a sulfonic acid derivative selected from the class consisting of an alkyl sulfonic acid and an aryl sulfonic acid as a curing agent, applying the composition in a configuration of a selected design, and curing the composition after application to said finished paper.

2. A method for making chemical watermarks in finished paper products which includes the steps of applying to the surface of finished paper a composition having curable hexamethoxymethylmelamine, a curing agent therefor which is a sulfonic acid derivative selected from the class consisting of an alkyl sulfonic acid and an aryl sulfonic acid, and a colorless organic polar solvent, applying said composition in the configuration of a selected design, and curing the composition in the paper after application to said finished paper, whereby a colorless, substantially insoluble chemical watermark is formed.

3. The method according to claim 2 further characterized by and including the step of evaporating the solvent after the composition has been applied in the configuration of a selected design.

4. The method according to claim 2 further characterized in that the composition is applied to the surface of the finished paper substantially at room temperature and the composition cures at substantially room temperature.

5. The method according to claim 2 further characterized by and including the step of aging the applied watermark until substantial insolubility of the chemical watermark is attained.

6. A method for making a colorless, substantially insoluble chemical watermark in finished paper which includes the steps of applying to the surface of the paper a

composition having curable hexamethoxymethylmelamine, a curing agent therefor which is at least about 3 percent by weight of an alkyl substituted phenyl sulfonic acid, and at least about 40 percent by weight of a colorless polar organic solvent, applying said composition in the configuration of a selected design, and curing the composition in the paper after application to said finished paper.

7. The method according to claim 6 further characterized by and including the step of aging the applied composition in the paper until substantial insolubility of the chemical watermark is attained.

8. A method for making a colorless, substantially insoluble chemical watermark in finished paper which includes the steps of applying to the surface of the paper a composition having hexamethoxymethylmelamine, a curing agent therefor which is at least about 3 percent by weight of a toluene sulfonic acid, and at least about 40 percent by weight of diethyleneglycol monomethyl ether, applying said composition in the configuration of a selected design, and curing the composition after application to said paper.

9. A method for making a chemical watermark in finished paper which includes the steps of applying to the surface of the finished paper a composition having hexamethoxymethylmelamine, an epoxy resin, an alkyl substituted phenyl sulfonic acid curing agent for the hexamethoxymethylmelamine in the configuration of a selected design, and curing the composition in the paper whereby a colorless, substantially insoluble chemical watermark is formed.

10. A method according to claim 9 further characterized by and including the step of aging the applied watermark until substantial insolubility of the chemical watermark is attained.

#### References Cited by the Examiner

#### UNITED STATES PATENTS

40 3,140,959 7/1964 Vaurio ----- 117-38

WILLIAM D. MARTIN, Primary Examiner.

H. W. MYLIUS, Assistant Examiner.